

# United States Patent Office

2,702,768  
Patented Feb. 22, 1955

1

2,702,768

## FERROUS SURFACE COATING PROCESS USING ALKALI METAL PHOSPHATES AND HY- DROXYLAMINES

Montagu Hyams and Andrew Nicholson, London, Eng-  
land, assignors to Parker Rust-Proof Company, Detroit,  
Mich., a corporation of Michigan

No Drawing. Original application July 21, 1949, Serial  
No. 106,103, now Patent No. 2,657,156, dated October  
27, 1953. Divided and this application March 26,  
1953, Serial No. 344,904

3 Claims. (Cl. 148—6.15)

This invention relates to the coating of ferrous surfaces  
to improve their resistance to corrosion.

The resistance to corrosion of ferrous surfaces can be  
improved by treating said surfaces with solutions of acid  
metal phosphates of metals such as zinc, manganese,  
cadmium, iron, calcium and barium. In these processes  
phosphate coatings are formed on the ferrous surface, and  
the metal present in the acid metal phosphate contained  
in the coating solution enters into the protective coating.  
These phosphates have, therefore, been described as  
"coating phosphates," i. e. phosphates in which the metal  
present enters into the protective coating.

In British Patent No. 517,049 it is disclosed that pro-  
tective coatings can be produced rapidly on ferrous  
surfaces by treatment with a solution which is primarily  
one of phosphoric acid or a "non-coating phosphate,"  
i. e. a phosphate in which the metal present does not enter  
into the protective coating, or both and which also con-  
tains a small amount of a nitrite, nitrate or sulphite, but  
which contains at the most only a small quantity of ions  
of metals which form coating phosphates.

The present invention is based on the discovery that  
in non-coating phosphate solutions improved results are  
obtained by using, instead of nitrite, nitrate or sulphite  
as taught in British Patent 517,049, hydroxylamine and  
its salts.

It is characteristic of hydroxylamine and its salts that  
coatings are produced in their presence, when used in  
conjunction with a solution which is primarily one of a  
"non-coating phosphate" and phosphoric acid and which  
contains at the most only a small quantity of ions of  
metals which form "coating phosphates," that are of a  
quality or density distinct from and superior to those  
obtainable from the use of such solutions by themselves  
even after extremely long times of treatment. By their  
action a coating of increased thickness is formed, which  
is exactly the opposite of the effect of suitable reducible  
compounds with "coating phosphates," and the reducible  
compounds of this invention are therefore to be regarded  
not as accelerators but as being vital for the coating  
process.

It is to be appreciated that small amounts of iron and  
other metal accelerators may be added to the solution, as  
described below but in any event a small amount of ions  
of metals which form coating phosphates will invariably  
be present after the solution has been in use for some  
time, for on treating ferrous surfaces with the solutions  
of the invention iron partly dissolves. However, the  
conditions are so controlled that the quantity of "coating  
phosphate" present in solution is extremely low since, in  
order that a suitable coating may be produced upon the  
ferrous surface the pH of the solution must be sufficiently  
high to favour the precipitation of a ferrous phosphate  
no less basic than the tertiary phosphate because it has  
been found by us that ferrous secondary phosphate is  
unsuitable as a coating constituent, being rapidly con-  
verted to powdery ferric phosphate. It has further been  
found by us that only when ferrous tertiary phosphate is  
precipitated above 60° C. does it exist in a form which  
resists far better than any other the tendency to oxidise to  
ferric phosphate so that we have found that if maximum  
benefit of our invention is to be obtained the solutions  
must be used at temperatures exceeding 60° C. and at pH

2

values sufficiently high to satisfy the condition specified  
above. This minimum pH will depend upon many  
factors such as temperature and phosphate concentration  
but we have found from precipitation experiments that  
a minimum pH of 4.2 will ensure the required conditions.  
Lower pH values than this may well lead to very loose  
coatings and also to the presence of appreciable amounts  
of "coating phosphate" in solution.

On treating ferrous surfaces according to our invention  
iron dissolves incipiently from the surface and a pro-  
tective phosphate-containing coating is formed in which  
the metal radical present is derived from the metal being  
coated, the metal present in the "non-coating phosphate"  
remaining in solution. In order for this incipient dis-  
solution to take place no pH above a certain maximum  
for any particular combination of reducible compound  
and "non-coating phosphate" is permissible. It has been  
found that in order to derive maximum benefit from our  
invention this pH should not normally exceed 5.8 and  
with some combinations should preferably be less than  
this. The best pH range for each particular reducible  
compound will be a function of its concentration and  
temperature of use but all will be found to be most suit-  
able for use within the limits of pH 4.2—5.8.

25 Due to the low acidity of the bath dissolved iron is  
precipitated immediately as coating without forming more  
than a negligible amount of sludge. This means that  
chemical consumption, scaling of steam coils and clogging  
of spray jets are reduced to a minimum. Sludge is also  
far less than when "coating phosphates" are employed  
since "non-coating phosphates" do not precipitate out  
insoluble phosphate due to dissociation when heated or  
neutralised as do equilibrium solutions of "coating  
phosphates."

30 Examples of "non-coating phosphates" as specified  
above are those of the alkali metals such as the sodium  
and potassium phosphates, as well as those of ammonium.  
Mixtures of these phosphates may be employed. The  
"non-coating phosphates" are in many cases cheaper and  
more readily available than the "coating phosphates" and  
as explained above in using them no substantial amount  
of sludge is formed. A copper, nickel or other metal  
accelerator may be incorporated in the solution. The  
most suitable concentration of such phosphate for use has  
been found to lie within the range 0.05 to 0.25 molar.

35 The coating solutions of the invention may be sprayed  
on to the metal surface to be coated, or the metal may  
be immersed in the solution to which wetting agents or  
thickening agents may with advantage be added to  
50 facilitate the coating action.

Hydroxylamine and its salts have been found to be  
very suitable for use in the present invention, optimum  
concentrations being 0.1—0.5% in the case of the hydro-  
chloride.

55 Various well known oxidising agents such as perman-  
ganates have been found to be ineffective whilst others  
such as hydrogen peroxide and hypochlorite have been  
found to yield substantially nothing but dust when used  
in controllable amount. Organic reducible compounds  
60 such as trichloracetic acid and quinone, active in con-  
junction with "coating phosphates," were found to be  
ineffective for the purpose of the present invention.

If the compounds of this invention are used substan-  
65 tially below the lower limit of concentration recom-  
mended above the necessary change in coating quality or  
density over that obtainable without their use for maxi-  
mum benefit cannot be attained even after very prolonged  
70 periods of processing. If used substantially above the  
upper limit of concentration recommended above the  
compounds of the invention will cease to produce a coating  
of any description or yield mainly loose dust on the  
surface. Mixtures of suitable compounds may be used  
in which case their effect may be regarded as additive.

75 The precise concentration of suitable reducible com-  
pound recommended for use in any given situation will  
depend upon the temperature, pH and time of treatment.  
In general the higher the temperature and the longer the  
time of treatment the lower the concentration of hydrox-  
80 yamine required or desirable, whilst the reverse is true  
in the case of pH. Usually higher concentrations of

reducible material are permissible with consequently more efficient coating action in the presence of wetting agents, thickening agents or agitation of the solution. The general criterion in deciding the correct concentration of hydroxylamine for producing coatings on ferrous surfaces for the subsequent application of paints, lacquers or like materials is to select any concentration within the limits specified heretofore which will give a uniform adherent coating associated with not more than 10-20 mg./sq. ft. of loose coating.

The coatings of the invention, after rinsing in water and drying, are eminently suitable for use as a base for paints, lacquers or like materials and also for oils but it is of advantage to rinse the coatings produced with a dilute solution of chromic, phosphoric or oxalic acid, or with a dilute solution of an iron, chromium or aluminium salt, for instance ferrous sulphate, ferric nitrate, chromium sulphate or nitrate, or aluminium sulphate or nitrate, or with a solution containing a mixture of these substances prior to drying and the application of paints, lacquers, oils or like materials. The concentration of the rinsing solution is suitably from 7-21 ozs. of the acid or salt in 100 gallons of water, although more concentrated solutions may be employed, and the temperature of the rinsing solution is preferably from 150°-180° F. A rinsing period of one minute is satisfactory, and by the rinsing the resistance of the metal to corrosion is increased and the tendency of the paint applied to the coating to blister is reduced.

We have found that dilute solutions of chromic acid, or solutions containing hexavalent chromium, are particularly effective in this respect and give a most surprising increase in corrosion resistance. As little as 0.005% chromic acid in the rinse will bring about a marked improvement, but this improvement becomes even more marked as the concentration of chromic acid is increased up to around 0.25%. Beyond this concentration no substantial improvement in corrosion resistance is discernible whilst the coatings tend to become very stained. The most useful concentration of chromic acid for use with coatings of the invention has been found to lie between 0.02-0.1% Cr<sub>2</sub>O<sub>3</sub>, the rinsing solution preferably being applied for a period of up to one minute at 150°-180° F.

The invention is illustrated by the following example:

A solution was employed containing in 100 gallons of water, 15 lbs. of 75% phosphoric acid, 3 lbs. hydroxylamine hydrochloride and sufficient ammonium hydroxide to give a pH of 4.8.

The solution was placed in a spray machine and heated to about 170° F.-180° F. and sprayed onto the metal to be coated for a period of about one minute.

The metal surface after withdrawal from the processing solution was rinsed in hot water, followed by immersion for one-half minute in a solution of 10 ounces of chromic acid per 100 gallons of water maintained at 160° F., before final force drying.

By this treatment very dark, adherent, even, hard

corrosion-resistant coatings of some 150-200 mg./sq. ft. were obtained upon ferrous surfaces which were eminently suitable for use as a base for paints, lacquers or like materials.

The invention includes the novel treating solutions as well as their use in the treatment of metallic surfaces.

This application is a division of application, Serial No. 106,103, filed July 21, 1949, now U. S. Patent 2,657,156.

We claim:

10. 1. A process for the production of phosphate coatings on ferrous surfaces in which process the surface is treated with a coating solution consisting essentially of at least one substance selected from the group consisting of phosphoric acid, ammonium phosphate and the alkali metal phosphates, said phosphate being present in a concentration of 0.05 to 0.25 molar, hydroxylamine in the amount of 0.1 percent to 0.5 percent and the salts thereof in an equivalent concentration, said solution being maintained at a temperature above 60° C. and containing sufficient alkaline material to produce a pH within the range of 4.2 to 5.8.
15. 2. A liquid composition for the production of phosphate coatings on ferrous surfaces, said composition consisting of an aqueous solution consisting essentially of at least one substance selected from the group consisting of phosphoric acid, ammonium phosphate and the alkali metal phosphates, said phosphate being present in a concentration of from 0.05 to 0.25 molar, hydroxylamine in the amount of .1 percent to .5 percent and the salts thereof in an equivalent concentration, said solution containing sufficient alkaline material to produce a pH within the range of 4.2 to 5.8.
20. 3. A process for the production of phosphate coatings on ferrous surfaces which comprises the steps of treating the said surface with a coating solution consisting essentially of at least one substance selected from the group consisting of phosphoric acid, ammonium phosphate and the alkali metal phosphates, said phosphate being present in a concentration of 0.05 to 0.25 molar, hydroxylamine in an amount of 0.1%-0.5% and the salts thereof in an equivalent concentration, said solution being maintained at a temperature above 60° C. and containing sufficient alkaline material to produce a pH within the range of 4.2 to 5.8, continuing the treatment until a coating is formed and thereafter rinsing the coating in a dilute aqueous solution of chromic acid.
25. 35. 40. 45.

#### References Cited in the file of this patent

#### UNITED STATES PATENTS

|           |                       |               |
|-----------|-----------------------|---------------|
| 2,268,323 | Martin et al. -----   | Dec. 30, 1941 |
| 2,298,280 | Clifford et al. ----- | Oct. 13, 1942 |
| 2,403,426 | Douty et al. -----    | July 2, 1946  |

#### FOREIGN PATENTS

|         |                     |               |
|---------|---------------------|---------------|
| 517,049 | Great Britain ----- | July 18, 1940 |
| 519,823 | Great Britain ----- | Apr. 8, 1940  |